# EUROPEAN PATENT SPECIFICATION

(11) **EP 2 071 013 B1**
(45) Date of publication and mention of the grant of the patent: **08.11.2017**
(21) Application number: 08105917.2
(22) Date of filing: 02.12.2008
(51) Int. Cl.: C10M 169/04, C10N 20/02, C10N 20/04, C10N 30/08

(54) **Lubricant composition comprising a flow improver having a bi-modal side-chain distribution**
Schmiermittelzusammensetzung enthaltend einen Fliessverbesserer mit einem bimodalen Seitenkettenverteilung
Composition lubrifiante comprenant un agent d'amélioration de l'écoulement comportant une distribution de chaîne latérale bimodale

(30) Priority: 03.12.2007 US 949083
(43) Date of publication of application: 17.06.2009
(73) Proprietor: Infineum International Limited, Abingdon Oxfordshire OX13 6BB (GB)
(72) Inventor: Bloch, Ricardo, Linden, NJ 07036 (US); Boese, Doyle Harold, Linden, NJ 07036 (US); Martella, David, Linden, NJ 07036 (US)
(74) Representative: Goddard, Frances Anna

(56) References cited:
- EP-A1- 0 296 714
- EP-A2- 1 086 964
- WO-A1-98/28386
- GB-A- 635 903
- JP-A- 10 310 758

## Description

### FIELD OF THE INVENTION

The present invention relates to lubricant compositions having improved flow properties, particularly lubricant compositions comprising American Petroleum Institute (API) Group III base stocks which exhibit improved low temperature flow properties.

### BACK GROUND OF THE INVENTION

Lubricant compositions are used in various applications such as automotive applications, industrial applications, etc. Lubricant compositions are typically formulated from a base stock and one or more additives.

Various additives for use in lubricant compositions are well known in the art. Examples of such additives include, but are not limited to, lube oil flow improvers (LOFIs), viscosity modifiers (VMs), etc.

Automobile manufacturers and government regulators have introduced new, more stringent performance requirements for lubricants. Examples are the requirements for oil volatility and fuel efficiency. These changes have made the choice of base stock(s) used in lubricants much more important than they were in the past. Due to their low viscosity and low volatility, API Group III base stocks have become the base stock of choice for the next generation of lubricant compositions.

WO98/28386A, EP 0,296,714 A and GB 635,903 A disclose (di)alkyl fumarate-vinyl acetate copolymers for use as a lube oil flow improver.

The present invention provides a lubricant composition having improved low temperature flow performance properties comprising (a) an API Group III base stock; (b) a semi-crystalline viscosity modifier; and (c) one or more LOFIs having a side-chain distribution which satisfies certain requirements.

### SUMMARY OF THE INVENTION

According to a first aspect, the present invention provides a lubricant composition comprising (a) an API Group III base stock;
(b) one or more semi-crystalline viscosity modifier(s) which is a copolymer of ethylene copolymerized with at least one additional alphaolefin monomer having from 3 to 30 carbon atoms; and
(c) one or more LOFIs which is a dialkyl fumarate-vinyl acetate copolymer having a side-chain distribution which satisfies the following requirements:
   (1) the distribution contains side chains ranging from C₈ to C₁₈ with an average carbon number ranging from 12.4 to 14.4;
   (2) the side chain distribution is bi-modal with a lower portion of the bi-modal distribution made up primarily of C₁₂ and an upper portion of the distribution made up primarily of C₁₆, C₁₈ or combinations thereof;
   (3) the total mole % of the upper portion of the distribution must be less than that of the lower portion of the distribution;
   (4) the amount of C₁₄ on the side chain is less than 20 mole % of the total side chain distribution when the essential components of the bi-modal distribution is made up of mixtures of (i) C₁₂ and C₁₆ or (ii) C₁₂, C₁₆ and C₁₈; and,
   (5) the amount of C₁₂ on the side chain must be at least 40 mole % of the total side chain distribution.

Suitably, the lubricant composition comprises an automotive lubricating oil composition, more especially an automotive lubricating oil composition for use in piston engines, especially gasoline (spark-ignited) and diesel (compression-ignited), crankcase lubrication, such compositions being referred to as crankcase lubricants.

According to a second aspect, the present invention provides a method of lubricating a compression-ignited or spark-ignited combustion engine, comprising operating the engine with a lubricant composition according to the first aspect of the invention.

Preferably, the method according to the second aspect of the present invention comprises lubricating the crankcase of a compression-ignited or spark-ignited internal combustion engine.

According to a third aspect, the present invention provides the use, in a lubricant composition which comprises an API Group III base stock, of (b) a semi-crystalline viscosity modifier as defined in accordance with the first aspect of the
present invention; in combination with (c) one or more LOFIs as defined in accordance with the first aspect of the present invention, to improve the low temperature flow properties of the lubricant composition.

Suitably, the low temperature flow properties of the lubricant composition are measured using the MRV Pumpability Test according to ASTM D4684. Suitably, the use in accordance with the third aspect of the present invention enables the lubricant composition to pass the MRV Pumpability Test according to ASTM D4684.

It will be appreciated that the term "lubricant composition" as used herein represents a "lubricating oil composition".

### DETAILED DESCRIPTION OF THE INVENTION

The features of the invention relating, where appropriate, to each and all aspects of the invention, will now be described in more detail as follows:
Unless otherwise indicated, all numbers expressing quantities of ingredients, reaction conditions, dimensions, physical characteristics, processing parameters, and the like, used in the specification and claims are to be understood as being modified in all instances by the term "about". Accordingly, unless indicated to the contrary, the numerical values set forth in the following specification and claims may vary depending upon the desired properties sought to be obtained by the present invention. At the very least, each numerical value should at least be construed in light of the number of reported significant digits and by applying ordinary rounding techniques. Moreover, all ranges disclosed herein are to be understood to encompass the beginning and ending range values and any and all subranges subsumed therein. For example, a stated range of "1 to 10" should be considered to include any and all subranges between (and inclusive of) the minimum value of 1 and the maximum value of 10; that is, all subranges beginning with a minimum value of 1 or more and ending with a maximum value of 10 or less, e.g., 5.5 to 10.

As used herein, the following terms are defined in the manner described below.

The term "polymer" includes copolymers unless otherwise specifically stated to be limited to a polymer derived solely from the polymerization of a single monomer and encompasses branched as well as linear polymers.

The term "copolymer" refers to a polymer resulting from the polymerization reaction of two chemically different monomers. With reference to ethylene alphaolefin copolymers, it is understood that such copolymers can optionally contain a minor amount (for example, greater than zero but less than 10% by weight) of a nonconjugated polyene, in which case the copolymer is sometimes referred to as a terpolymer. With reference to ethylene alphaolefin polymers, it is understood both copolymers and terpolymers of ethylene with at least one other alpha-olefin are included.

The term "average carbon number" refers to the average carbon number weighted by molar fraction.

The term "lubricating oil flow improver" (LOFI) covers all additives which modify the size, number, and growth of wax crystals in lubricating (or lube for short) oils in such a way as to impart improved low temperature handling, pumpability, and/or vehicle operability as measured by such tests as pour point, Mini-Rotary Viscometer (MRV), and Scanning Brookfield Viscometer. The majority of lubricating oil flow improvers are polymers or copolymers, or contain polymers or copolymers. These polymers are generally side chain, backbone or mixtures thereof.

The term "base oil" refers to a refined fluid that is free of additives and is used as a component in a lubricant blend.

The term "base stock" refers to a blend, mixture, or similar of base oils.

Various "Groups" of base stocks, for example, API Group III base stocks, will be referred to herein. Those Group classifications have been established by the American Petroleum Institute (API) according to the table included in U.S. Patent No. 6,475,963.

The term "bi-modal" refers to a carbon chain length frequency distribution which has two distinct peaks (or modes) with each peak being a carbon chain length (or carbon chain lengths adjacent in terms of sequential even number of carbons) which has a higher mole percentage than neighboring carbon chain lengths. The bi-modal carbon chain length frequency distribution has a "lower portion of the distribution" and an "upper portion of the distribution".

The term "lower portion of the distribution" refers to the portion of the bi-modal distribution which is composed of the mode with the lower carbon chain length (or lengths) and adjacent carbon chain lengths (in terms of sequential even number chain lengths) of lower mole percent. The highest carbon chain length in the lower portion of the distribution is C₁₄.

The term "upper portion of the distribution" refers to the portion of the bi-modal distribution which is composed of the mode with the higher carbon chain length (or lengths) and adjacent carbon chain lengths of lower mole percent. The lowest carbon chain length in the upper portion of the distribution is C₁₆.

The term "primarily" means the amount of one component present in the composition, compound, etc. is more than the amounts of any other component present on a component-by-component basis.

The lubricant composition comprises (a) a Group III base stock; (b) a semi-crystalline viscosity modifier; and (c) one or more LOFIs that meet certain specifications.

The lubricant composition comprises an API Group III base stock. Group III base stocks as defined by the API have a viscosity index that is open-ended. Suitably, the viscosity index of the base stock is greater than 120. Alternatively, the base stocks has a viscosity index of equal to or greater than 120 and equal to or less than 200. Suitable, commercially available Group III base stocks include, but are not limited to: the Visom brand of base stocks commercially available from ExxonMobil (Fawley, U.K.); the Yubase brand of base stocks commercially available from SK Corporation (Ulsan, South Korea); the Ultra-S brand of base stocks are commercially available from ConocoPhillips (Westlake, LA (USA)); and the Nexbase brand of base stocks commercially available from Neste (Porvoo, Finland).

Suitably, the base stock is made using gas-to-liquids ("GTL") process. GTL is a refinery process used to convert natural gas or other gaseous hydrocarbons into longer-chain hydrocarbons. For example, GTL can be used to convert methane-rich gases into liquid fuels either via direct conversion or via syngas as an intermediate using the Fischer Tropsch process. As is well known in the art, isomerization catalyst can be used with GTL to make Group III base stocks

The lubricant composition comprises a semi-crystalline viscosity modifier. Typically, the semi-crystalline viscosity modifier comprises one or more high molecular weight hydrocarbon polymers as is well known in the art. Examples of suitable hydrocarbon polymers include copolymers of ethylene copolymerized with at least one additional alphaolefin monomer having from 3 to 30, for example, from 3 to 8 carbon atoms and which may be straight or branched. Optionally, a low concentration, e.g., less than about 10 wt. %, of a nonconjugated diene can be present. In a non-limiting embodiment, these copolymers are those comprising ethylene and propylene. Ethylene copolymers suitable for the present invention include tapered or block copolymers (including terpolymers, tetrapolymers, etc.) as well as those that have controlled compositional homogeneity and/or heterogeneity within and among copolymer chains which are well known in the art. Such copolymers are described in "Polymers as Lubricating Oil Viscosity Modifiers", G. VerStrate, M. J. Struglinski, Chapter 15; in "Polymers as Rheology Modifiers", D. N. Schulz and J. E. Glass, editors, American Chemical Society, Washington, D.C., 1991.

Suitably, the semi-crystalline viscosity modifier is an oil-soluble polymer comprised of ethylene and a C₃ to C₁₈ alpha-olefin, the polymer being characterized by the following combination of parameters: (a) an average ethylene content within the range between 60 to 80 mole percent, wherein said polymer contains no more than 1.3% by weight of a polymer fraction which is insoluble in normal decane at 45°C; (b) a degree of crystallinity less than 25%; (c) a weight average molecular weight/number average molecular weight ratio less than 4.0; and (d) a viscosity average molecular weight within the range between 10,000 and 200,000 Daltons. Suitable viscosity modifiers are disclosed in US Patent No. 3,551,336.

Alternatively, the semi-crystalline viscosity modifier is a segmented copolymer of ethylene and at least one other alpha-olefin monomer; each copolymer is intramolecularly heterogeneous and intermolecularly homogeneous and at least one segment of the copolymer, constituting at least 10% of the copolymer's chain, is a crystallizable segment. Suitable viscosity modifiers are disclosed in US Patent No. 4,804,794.

Suitably, the semi-crystalline viscosity modifier is included in combination with an amorphous viscosity modifier. An example of this is an oil-soluble polymer composition comprising a first copolymer of ethylene and a C₃ to C₁₈ alpha-olefin having an ethylene content of 50-95 mole percent and a second copolymer of ethylene and a C₃ to C₁₈ higher alpha-olefin having an ethylene content of 5-80 mole percent, the ethylene content of the first copolymer being at least 5 mole percent more than the ethylene content of the second polymer. Suitable amorphous viscosity modifiers are disclosed in US Patent No. 3,697,429.

Suitably, the semi-crystalline viscosity modifier has a number average molecular weight ranging from 20,000 to 500,000 Daltons, for example, from 25,000 to 400,000 Daltons or from 30,000 to 300,000 Daltons as determined by gel permeation chromatography.

The semi-crystalline viscosity modifier can be present in the lubricant composition in an amount ranging from 0.05 to 5 wt. % of the polymer

The lubricant composition comprises one or more LOFIs having a side-chain distribution which satisfies the following requirements:
(1) Every side chain present comprises carbon chains made up of from 8 to 18 carbon atoms with an average carbon number from 12.4 to 14.4, for example, from 12.8 to 14.0 or from 13.0 to 13.8;
(2) the side chain distribution is bi-modal with the lower portion of the bi-modal distribution made up primarily of C₁₂ and the upper portion of the distribution (i.e., the distribution with the higher carbon number mode) made up primarily of C₁₆, C₁₈ or combinations thereof;
(3) the total mole % of the upper portion of the distribution must be less than that of
   the lower portion of the distribution; and
(4) the amount of C₁₂ on the side chain must be at least 40 mole %, for example, at least 50 mole % or at least 60 mole %, of the total side chain distribution.

Suitably, when the essential components of the bi-modal distribution are made up of mixtures of (a) C₁₂ and C₁₆ or (b) C₁₂, C₁₆ and C₁₈, the amount of C₁₄ must be less than 20 mole %, for example, less than 10 mole % of the total side chain distribution.

Suitably, the side chains comprise even carbon number segments ranging from C₈ to C₁₈, i.e., C₈, C₁₀, C₁₂, C₁₄, C₁₆, C₁₈.

Suitably, the LOFI comprises a dialkyl fumarate-vinyl acetate copolymer.

The dialkyl fumarate-vinyl acetate copolymer can be formed from a mixture of alcohols having carbon numbers ranging from 8 to 18, with an average carbon number from 12.4 to 14.4, for example, from 12.8 to 14.0, or from 13.0 to 13.8. The copolymer is a sidechain copolymer having methylene segments as the side chains.

These LOFIs can contain pendent ester groups derived from a mixture of alcohols whereby the alcohol residue can be characterized as repeating methylene units, and which are oil soluble, or dispersible, polymeric compositions that generally have weight average molecular weights ranging from 50,000 to 350,000 Daltons as determined by gel permeation chromatography.

Suitably, the dialkyl fumarate-vinyl acetate copolymer has a specific viscosity ranging from 0.3 to 1.5, for example, from 0.3 to 1.0 or from 0.45 to 0.7. Suitably, the dialkyl fumarate-vinyl acetate copolymer has a weight average molecular weight ranging from 50,000 to 350,000 Daltons, for example, from 50,000 to 200,000 Daltons or from 75,000 to 120,000 Daltons.

The LOFI and one or more other components, excluding the base stock, in a lubricant composition are referred to as "additives".

Suitably, the LOFI has a weight average molecular weight, as determined by gel permeation chromatography, ranging from 50,000 to 350,000 Daltons, for example from 80,000 to 200,000 Daltons.

Suitably, the LOFI has a specific viscosity ranging from 0.3 to 1.0, for example, from 0.4 to 0.8.

The LOFI can be present in the lubricant composition in an amount ranging from 0.005 to 1.0 weight percent, for example from 0.05 to 0.5 weight percent.

The lubricant composition of the present invention can further comprise one or more of the optional components: corrosion inhibitors, oxidation inhibitors, friction modifiers, dispersants, anti-foaming agents, anti-wear agents, detergents, rust inhibitors, etc.

Suitably, the lubricant composition of the present invention comprises a corrosion inhibitor. Corrosion inhibitors, also known as anti-corrosive agents, reduce the degradation of the metallic parts contacted by the lubricating oil composition. Illustrative of corrosion inhibitors are phosphosulfurized hydrocarbons and the products obtained by reaction of a phosphosulfurized hydrocarbon with an alkaline earth metal oxide or hydroxide, preferably in the presence of an alkylated phenol or of an alkylphenol thioester, and also preferably in the presence of carbon dioxide. Phosphosulfurized hydrocarbons are prepared by reacting a suitable hydrocarbon such as a terpene, a heavy petroleum fraction of a C₂ to C₆ olefin polymer such as polyisobutylene, with from 5 to 30 wt. percent of a sulfide of phosphorus for 1/2 to 15 hours, at a temperature in the range of 150°F to 600°F (66°C to 316°C). Neutralization of the phosphosulfurized hydrocarbon may be effected in the manner taught in U.S. Pat. No. 1,969,324.

Suitably, the lubricant composition of the invention can comprise an oxidation inhibitor. Oxidation inhibitors reduce the tendency of mineral oils to deteriorate in service which deterioration can be evidenced by the products of oxidation such as sludge and varnish-like deposits on the metal surfaces, and by viscosity growth. Such oxidation inhibitors include alkaline earth metal salts of alkylphenolthioesters having preferably C₅ to C₁₂ alkyl side chains, e.g., calcium nonylphenol sulfide, barium t-octylphenyl sulfide, dioctylphenylamine, phenylalphanaphthylamine, phosphosulfurized or sulfurized hydrocarbons, etc.

Suitably, the lubricant of the present invention comprises a friction modifier. Friction modifiers serve to impart the proper friction characteristics to lubricating oil compositions such as automatic transmission fluids. Representative examples of suitable friction modifiers are found in U.S. Pat. No. 3,933,659 that discloses fatty acid esters and amides; U.S. Pat. No. 4,176,074 that describes molybdenum complexes of polyisobutenyl succinic anhydride-amino alkanols; U.S. Pat. No. 4,105,571 that discloses glycerol esters of dimerized fatty acids; U.S. Pat. No. 3,779,928 that discloses alkane phosphonic acid salts; U.S. Pat. No. 3,778,375 that discloses reaction products of a phosphonate with an oleamide; U.S. Pat. No. 3,852,205 that discloses S-carboxyalkylene hydrocarbyl succinimide, S-carboxyalkylene hydrocarbyl succinamic acid and mixtures thereof; U.S. Pat. No. 3,879,306 that discloses N-(hydroxyalkyl)alkenyl-succinamic acids or succinimides; U.S. Pat. No. 3,932,290 which discloses reaction products of di-(lower alkyl) phosphites and epoxides; and U.S. Pat. No. 4,028,258 that discloses the alkylene oxide adduct of phosphosulfurized N-(hydroxyalkyl) alkenyl succinimides. Preferred friction modifiers include succinate esters, or metal salts thereof, of hydrocarbyl substituted succinic acids or anhydrides and thiobis alkanols such as described in U.S. Pat. No. 4,344,853 as well as various molybdenum compounds.

Suitably, the lubricant composition of the present invention comprises a dispersant. Dispersants maintain compounds resulting from oxidation during use that are insoluble or substantially insoluble in the oil, in suspension in the fluid thus preventing sludge flocculation and precipitation or deposition on metal parts. Suitable dispersants include high molecular weight alkyl succinates, the reaction product of oil-soluble polyisobutylene succinic anhydride with ethylene amines such as tetraethylene pentamine and borated salts thereof.

Suitably, the lubricant composition of the present invention comprises a component to provide foam control. Foam control can be provided by an antifoamant of the polysiloxane type, e.g., silicone oil and polydimethyl siloxane.

Suitably, the lubricant composition of the present invention comprises an anti-wear agent. Anti-wear agents, as their name implies, reduce wear of metal parts. Representatives of conventional anti-wear agents are zinc dialkyldithiophosphate and zinc diaryldithiophosphate.

Suitably, the lubricant composition of the present invention comprises a detergent and metal rust inhibitor. Detergents and metal rust inhibitors include the metal salts of sulphonic acids, alkyl phenols, sulfurized alkyl phenols, alkyl salicylates, naphthenates and other oil soluble mono- and dicarboxylic acids. Highly basic (viz., overbased) metal salts, such as highly basic alkaline earth metal sulfonates (especially Ca and Mg salts) are frequently used as detergents. Representative examples of such materials, and their methods of preparation, are found in U.S. Pat. No. 6,127,321.

The lubricant composition of the present invention can be made using methods and techniques which are well known in the art. Lubricant compositions according to the present invention are typically made by blending individual components into the base stock. For example, the components can be added directly to the base stock by dispersing, or dissolving the additives at the desired level of concentration at room temperature or elevated temperatures.

### Examples

The present invention is illustrated by the following non-limiting examples. In the Examples, the lubricant compositions comprised a Group III base stock (Yubase base stock); a semi-crystalline viscosity modifier (Paratone 8451 from Chevron Oronite Company); and a LOFI which was prepared as described below. Each lubricant composition contained a different LOFI. For example, the lubricant composition of Example 1 contains LOFI 1, the lubricant composition of Example 2 contains LOFI 2 and so on.

Five LOFIs (LOFIs 1-5) were prepared by first making five dialkyl fumarate monomers (Dialkyl Fumarate Monomers 1-5) using a blend of alcohols having a distribution of carbon atoms as shown in Table I. Alcohol 1 in Table I is used to prepare Dialkyl Fumarate Monomer 1, Alcohol 2 in Table I is used to prepare Dialkyl Fumarate Monomer 2 and so on. 232 g of fumaric acid, 824 g of the specified alcohol blend, and 0.2 g Fascat 4100® were added to the round bottom flask equipped with a Dean-Stark apparatus. The slurry was stirred under a stream of nitrogen and slowly heated to 220°C. The esterification reaction was monitored by measuring the amount of water collected in the Dean-Stark trap. When the evolution of water ceased (typically 4 to 6 hours), the dialkyl fumarate monomer was decanted from the reactor and analyzed for neutralization number (2.0 mg KOH/g) and saponification number (223 mg KOH/g). Dialkyl Fumarate Monomers 1-5 were formed in this way.

The LOFIs were then prepared by making a dialkyl fumarate-vinyl acetate copolymer from the dialkyl fumarate monomers (formed in the step described above) as described below. Dialkyl Fumarate Monomer 1 was used to prepare Dialkyl Fumarate Vinyl Acetate Copolymer 1, Dialkyl Fumarate Monomer 2 was used to prepare Dialkyl Fumarate Vinyl Acetate Copolymer 2 and so on. 150 g of a Dialkyl Fumarate Monomer (Dialkyl Fumarate Monomers 1-5) were added to a Parr® brand, 300 cm³ stainless steel reactor. The reactor was sealed, heated to 50°C, and flushed with nitrogen for 10 minutes. Then, 26.5 g of deoxygenated vinyl acetate were injected into the Parr® reactor containing the Dialkyl Fumarate Monomer. The mixture was stirred for 15 minutes before heating to the reaction temperature of 100°C. 0.26 g *tert*-butyl peroctoate was dissolved in 2.0 g Blandol® White Mineral Oil produced by Sonneborn and then injected into the mixture. The mixture was stirred for 5 to 8 hours to complete the polymerization reaction. The copolymer was then poured from the reactor into a round-bottom flask and stripped of volatiles on a rotary evaporator. Dialkyl Fumarate Vinyl Acetate Copolymers 1-5 were formed in this way.

Dialkyl Fumarate Vinyl Acetate Copolymers 1-5 were blended as is well known in the art with a Group III base stock (Yubase base stock) and a semi-crystalline viscosity modifier (Paratone 8451 from Chevron Oronite Company) to form the SAE 5W-30 lubricant compositions of Examples 1-5.

In Table I below, compositional information is provided for the LOFI Side Chains for Examples 1-5.

**Table I. Distribution of Carbon Atoms in Alcohols 1-5**

| | **Alcohol 1** | **Alcohol 2** | **Alcohol 3** | **Alcohol 4** | **Alcohol 5** |
|---|---|---|---|---|---|
| **C₈ [mole fraction]** | 0 | 0 | 0 | 0 | .1 |
| **C₁₀ [mole fraction]** | 0 | 0 | .2 | 0 | .3 |
| **C₁₂ [mole fraction]** | .7 | .708 | .5 | .4 | 0 |
| **C₁₄ [mole fraction]** | .1 | .084 | 0 | .5 | 0 |
| **C₁₆ [mole fraction]** | 0 | .008 | 0 | .1 | .6 |
| **C₁₈ [mole fraction]** | .2 | .200 | .3 | 0 | 0 |
| **Avg Cₙ** | 13.4 | 13.4 | 13.4 | 13.4 | 13.4 |

As stated previously, side chains of the LOFIs of the present invention must satisfy certain requirements. The various requirements are listed in Table II below. For the various exemplary lubricant compositions (Exs. 1-5) made in the manner described above, a "✔" appears in a box if the LOFI meets the requirement, and an "X" appears in a box if the LOFI does not meet the requirement.

**Table II**

| **Requirement** | **Ex. 1** | **Ex. 2** | **Ex. 3** | **Ex. 4** | **Ex. 5** |
|---|---|---|---|---|---|
| (1) the distribution contains side chains ranging from C₈ to C₁₈ with an average carbon number from 12.4 to 14.4 | ✔ | ✔ | ✔ | ✔ | ✔ |
| (2) the side chain distribution is bi-modal with the lower portion of the bi-modal distribution made up primarily of C₁₂ and the upper portion of the distribution made up primarily of C₁₆, C₁₈ or combinations thereof | ✔ | ✔ | ✔ | **X** | **X** |
| (3) the sum of the upper portion of the distribution must be less than the lower portion of the distribution. This necessitates the amount of C₁₄ must be less than 20% or less than 10% when the essential components of the bi-modal distribution are made up of mixtures of (a) C₁₂ and C₁₆ or (b) C₁₂, C₁₆ and C₁₈ and must be less than the sum of C₁₆ and C₁₈; | ✔ | ✔ | ✔ | **X** | **X** |
| (4) the amount of C₁₂ must be at least 40 mole % or at least 50 mole % of the total side chain distribution. | ✔ | ✔ | ✔ | ✔ | **X** |

As you can see, the LOFIs in the lubricant compositions of Examples 1-3 satisfy all of the requirements and are encompassed by the present invention. The LOFIs in the lubricant compositions of Examples 4 and 5 do not satisfy all of the requirements and fall outside of the present invention.

The lubricant compositions of Examples 1-5 were subjected to MRV Pumpability Test according to ASTM D 4684. The results of the test are shown in Table III.

**Table III. MRV Pumpability Test**

| | **Ex. 1** | **Ex. 2** | **Ex. 3** | **Ex. 4** | **Ex. 5** |
|---|---|---|---|---|---|
| **At a Treat Rate of 0.50%** | | | | | |
| Viscosity [mPa·s] | 27,200 | -- | 24,400 | 161,100 | 54,200 |
| Yield Stress [Pa] | < 35 | -- | < 35 | < 350 | <140 |

| **At a Treat Rate of 0.20%** | | | | | |
|---|---|---|---|---|---|
| Viscosity [mPa·s] | 23,800 | 21,400 | 22,400 | -- | -- |
| Yield Stress [Pa] | < 35 | < 35 | < 35 | -- | -- |

| | | | | | |
|---|---|---|---|---|---|
| -- means yield stress and viscosity were not tested. | | | | | |

In order to pass the MRV Pumpability Test, a lubricant composition must exhibit a viscosity equal to or less than 60,000 mPa·s and a yield stress of less than 35 Pa. At a treat rate of 0.50%, only Examples land 3 passed the MRV Pumpability Test. At a treat rate of 0.20%, only Examples 1-3 pass the MRV Pumpability Test. As stated above, Examples 1-3 are encompassed by the present invention.

## Claims

1. A lubricant composition comprising:
(a) an API Group III base stock;
(b) one or more semi-crystalline viscosity modifier(s) which is a copolymer of ethylene copolymerized with at least one additional alphaolefin monomer having from 3 to 30 carbon atoms; and
(c) one or more LOFIs which is a dialkyl fumarate-vinyl acetate copolymer having a side-chain distribution which satisfies the following requirements:
(1) the distribution contains side chains ranging from C₈ to C₁₈ with an average carbon number ranging from 12.4 to 14.4;
(2) the side chain distribution is bi-modal with a lower portion of the bi-modal distribution made up primarily of C₁₂ and an upper portion of the distribution made up primarily of C₁₆, C₁₈ or combinations thereof;
(3) the total mole % of the upper portion of the distribution must be less than that of the lower portion of the distribution;
(4) the amount of C₁₄ on the side chain is less than 20 mole % of the total side chain distribution when the essential components of the bi-modal distribution is made up of mixtures of (i) C₁₂ and C₁₆ or (ii) C₁₂, C₁₆ and C₁₈; and,
(5) the amount of C₁₂ on the side chain must be at least 40 mole % of the total side chain distribution.

2. The lubricant composition according to claim 1, wherein the distribution contains side chains ranging from C₈ to C₁₈ with an average carbon number ranging from 12.8 to 14.0.

3. The lubricant composition according to any one of the preceding claims, wherein the amount of C₁₄ on the side chain is less than 10 mole % of the total side chain distribution and the bi-modal distribution is made up of mixtures of (i) C₁₂ and C₁₆ or (ii) C₁₂, C₁₆ and C₁₈.

4. The lubricant composition according to any one of the preceding claims, wherein the amount of C₁₂ on the side chain must be at least 50 mole % of the total side chain distribution.

5. The lubricant composition according to any one of the preceding claims, wherein the side chains comprise even carbon number segments ranging from C₈ to C₁₈.

6. The lubricant composition according to any one of the preceding claims, wherein the dialkyl fumarate-vinyl acetate copolymer has a weight average molecular weight of from 50,000 to 350,000 Daltons.

7. The lubricant composition according to any one of the preceding claims, wherein the dialkyl fumarate-vinyl acetate copolymer has a specific viscosity ranging from 0.3 to 1.0.

8. The lubricant composition according to any one of the preceding claims, wherein the LOFI is present in an amount ranging from 0.005 weight percent to 1.0 weight percent, based on the total weight of the lubricant composition.

9. The lubricant composition according to any one of the preceding claims, wherein the semi-crystalline viscosity modifier is a copolymer of ethylene copolymerized with propylene.

10. The lubricant composition according to any one of the preceding claims, wherein the semi-crystalline viscosity modifier comprises an ethylene alpha-olefin copolymer containing a small amount of one or more non-conjugated dienes.

11. The lubricant composition according to any one of the preceding claims, wherein the semi-crystalline viscosity modifier is present in an amount of 0.05 to 5 wt %, based on the total weight of the lubricant composition.

12. The lubricant composition according to any one of the preceding claims, wherein the semi-crystalline viscosity modifier is included in combination with an amorphous viscosity modifier.

13. The lubricant composition according to any one of the preceding claims further comprising one or more of the following components: corrosion inhibitors, oxidation inhibitors, friction modifiers, dispersants.

14. A method of lubricating a compression-ignited or spark-ignited combustion engine comprising operating the engine with a lubricant composition as claimed in any one of the preceding claims.

15. The use, in a lubricant composition which comprises an API Group III base stock, of (b) one or more semi-crystalline viscosity modifier(s) as defined in any one of claims 1 to 13; in combination with (c) one or more LOFIs as defined in any one of claims 1 to 13, to improve the low temperature flow properties of the lubricant composition.

## Patentansprüche

1. Schmiermittelzusammensetzung, die
a) ein Basismaterial aus API-Gruppe III,
b) einen oder mehrere halbkristalline Viskosizitätsmodifizierer, der bzw. die Copolymer aus Ethylen copolymerisiert mit mindestens einem zusätzlichen α-Olefinmonomer ist bzw. sind, das bzw. die von 3 bis 30 Kohlenstoffatome aufweisen, und
c) einen oder mehrere Schmierölfließverbesserer (LOFI(s)), der bzw. die Dialkylfumarat-Vinylacetat-Copolymer ist bzw. sind, der bzw. die eine Seitenkettenverteilung aufweisen, die die folgenden Erfordernisse erfüllt:
(1) die Verteilung enthält Seitenketten im Bereich von C₈ bis C₁₈ mit einer durchschnittlichen Kohlenstoffzahl im Bereich von 12,4 bis 14,4,
(2) die Seitenkettenverteilung ist bimodal, wobei ein unterer Teil der bimodalen Verteilung hauptsächlich aus C₁₂ zusammengesetzt ist und ein oberer Teil der Verteilung hauptsächlich aus C₁₆, C₁₈ oder Kombinationen davon zusammengesetzt ist,
(3) die Gesamtmolprozent des oberen Teils der Verteilung müssen weniger als die des unteren Teils der Verteilung betragen,
(4) die Menge an C₁₄ an der Seitenkette beträgt weniger als 20 Mol% der gesamten Seitenkettenverteilung, wenn die wesentlichen Komponenten der bimodalen Verteilung aus Mischungen von (i) C₁₂ und C₁₆ oder (ii) C₁₂, C₁₆ und C₁₈ zusammengesetzt sind, und
(5) die Menge an C₁₂ an der Seitenkette muss mindestens 40 Mol% der gesamten Seitenkettenverteilung betragen,
umfasst.

2. Schmiermittelzusammensetzung nach Anspruch 1, bei der die Verteilung Seitenketten im Bereich von C₈ bis C₁₈ mit einer durchschnittlichen Kohlenstoffzahl im Bereich von 12,8 bis 14,0 enthält.

3. Schmiermittelzusammensetzung nach einem der vorhergehenden Ansprüche, bei der die Menge an C₁₄ an der Seitenkette weniger als 10 Mol% der gesamten Seitenkettenverteilung beträgt und die bimodale Verteilung aus Mischungen von (i) C₁₂ und C₁₆ oder (ii) C₁₂, C₁₆ und C₁₈ besteht.

4. Schmiermittelzusammensetzung nach einem der vorhergehenden Ansprüche, bei der die Menge an C₁₂ an der Seitenkette mindestens 50 Mol% der gesamten Seitenkettenverteilung betragen muss.

5. Schmiermittelzusammensetzung nach einem der vorhergehenden Ansprüche, bei der die Seitenketten geradzahlige Kohlenstoffsegmente umfassen, die im Bereich von C₈ bis C₁₈ liegen.

6. Schmiermittelzusammensetzung nach einem der vorhergehenden Ansprüche, bei der das Dialkylfumarat-Vinylacetat-Copolymer ein Molekulargewicht (Gewichtsmittel) von 50.000 bis 350.000 Dalton aufweist.

7. Schmiermittelzusammensetzung nach einem der vorhergehenden Ansprüche, bei der das Dialkylfumarat-Vinylacetat-Copolymer eine spezifische Viskosität im Bereich von 0,3 bis 1,0 aufweist.

8. Schmiermittelzusammensetzung nach einem der vorhergehenden Ansprüche, bei der das LOFI in einer Menge im Bereich von 0,005 Ges.-% bis 1,0 Gew.-% vorliegt, bezogen auf das Gesamtgewicht der Schmiermittelzusammensetzung.

9. Schmiermittelzusammensetzung nach einem der vorhergehenden Ansprüche, bei der der halbkristalline Viskosizitätsmodifizierer ein Copolymer von Ethylen copolymerisiert mit Propylen ist.

10. Schmiermittelzusammensetzung nach einem der vorhergehenden Ansprüche, bei der der halbkristalline Viskosizitätsmodifizierer ein Ethylen-α-Olefin-Copolymer umfasst, das eine kleine Menge an einem oder mehreren nichtkonjugierten Dienen enthält.

11. Schmiermittelzusammensetzung nach einem der vorhergehenden Ansprüche, bei der der halbkristalline Viskosizitätsmodifizierer in einer Menge von 0,05 bis 5 Gew.-% vorliegt, bezogen auf das Gesamtgewicht der Schmiermittelzusammensetzung.

12. Schmiermittelzusammensetzung nach einem der vorhergehenden Ansprüche, bei der der halbkristalline Viskosizitätsmodifizierer in Kombination mit einem amorphen Viskosizitätsmodifizierer eingeschlossen ist.

13. Schmiermittelzusammensetzung nach einem der vorhergehenden Ansprüche, die ferner einen oder mehrere der folgenden Bestandteile umfasst: Korrosionsinhibitoren, Oxidationsinhibitoren, Reibungsmodifizierer und Dispergiermittel.

14. Verfahren zum Schmieren eines kompressionsgezündeten oder funkengezündeten Verbrennungsmotors, bei dem der Motor mit einer Schmiermittelzusammensetzung wie in einem der vorhergehenden Ansprüche beansprucht betrieben wird.

15. Verwendung von (b) einem oder mehreren halbkristallinen Viskosizitätsmodifizierer(n) wie in einem der vorhergehenden Ansprüche 1 bis 13 definiert in einer Schmiermittelzusammensetzung, die ein Basismaterial aus API-Gruppe III umfasst, in Kombination mit (c) einem oder mehreren LOFIs wie in einem der vorgehenden Ansprüche 1 bis 13 definiert zur Verbesserung der Tieftemperaturfließeigenschaften der Schmiermittelzusammensetzung.

## Revendications

1. Composition lubrifiante comprenant :
(a) une huile de base du groupe III API ;
(b) un ou plusieurs modificateurs de viscosité semi-cristallins qui est un copolymère d'éthylène copolymérisé avec au moins un monomère d'alphaoléfine supplémentaire ayant 3 à 30 atomes de carbone ; et
(c) un ou plusieurs LOFI qui est un copolymère fumarate de dialkyle-acétate de vinyle ayant une distribution de chaînes latérales qui satisfait les exigences suivantes :
(1) la distribution contient des chaînes latérales se situant dans la plage allant de C₈ à C₁₈ avec un nombre de carbones moyen se situant dans la plage allant de 12,4 à 14,4 ;
(2) la distribution de chaînes latérales est bi-modale avec une partie inférieure de la distribution bi-modale constituée de jusqu'à principalement C₁₂ et une partie supérieure de la distribution constituée principalement de jusqu'à C₁₆, C₁₈ ou une de leurs combinaisons ;
(3) le % en moles total de la partie supérieure de la distribution doit être inférieur à celui de la partie inférieure de la distribution ;
(4) la quantité de C₁₄ sur la chaîne latérale est de moins de 20 % en moles de la distribution de chaînes latérales totale quand les composants essentiels de la distribution bi-modale sont constitués de mélanges de (i) C₁₂ et C₁₆ ou (ii) de C₁₂, C₁₆ et C₁₈ ; et,
(5) la quantité de C₁₂ sur la chaîne latérale doit être d'au moins 40 % en moles de la distribution de chaîne latérale totale.

2. Composition lubrifiante selon la revendication 1, dans laquelle la distribution contient des chaînes latérales se situant dans la plage allant de C₈ à C₁₈ avec un nombre de carbones moyen se situant dans la plage allant de 12,8 à 14,0.

3. Composition lubrifiante selon l'une quelconque des revendications précédentes, dans laquelle la quantité de C₁₄ sur la chaîne latérale est inférieure à 10 % en moles de la distribution de chaîne latérale totale et la distribution bi-modale est constituée de mélanges de (i) C₁₂ et C₁₆ ou (ii) de C₁₂, C₁₆ et C₁₈.

4. Composition lubrifiante selon l'une quelconque des revendications précédentes, dans laquelle la quantité de C₁₂ dans la chaîne latérale doit être d'au moins 50 % en moles de la distribution de chaînes latérales totale.

5. Composition lubrifiante selon l'une quelconque des revendications précédentes, dans laquelle les chaînes latérales comprennent des segments de nombre de carbone uniformes se situant dans la plage allant de C₈ à C₁₈.

6. Composition lubrifiante selon l'une quelconque des revendications précédentes, dans laquelle le copolymère fumarate de dialkyle-acétate de vinyle a un poids moléculaire moyen en poids de 50000 à 350000 daltons.

7. Composition lubrifiante selon l'une quelconque des revendications précédentes, dans laquelle le copolymère fumarate de dialkyle-acétate de vinyle a une viscosité spécifique se situant dans la plage allant de 0,3 à 1,0.

8. Composition lubrifiante selon l'une quelconque des revendications précédentes, dans laquelle le LOFI est présent en une quantité se situant dans la plage allant de 0,005 pour cent en poids à 1,0 pour cent en poids, sur la base du poids total de la composition lubrifiante.

9. Composition lubrifiante selon l'une quelconque des revendications précédentes, dans laquelle le modificateur de viscosité semi-cristallin est un copolymère d'éthylène copolymérisé avec du propylène.

10. Composition lubrifiante selon l'une quelconque des revendications précédentes, dans laquelle le modificateur de viscosité semi-cristallin comprend un copolymère éthylène alpha-oléfine contenant une faible quantité d'un ou plusieurs diènes non conjugués.

11. Composition lubrifiante selon l'une quelconque des revendications précédentes, dans laquelle le modificateur de viscosité semi-cristallin est présent en une quantité de 0,05 à 5 % en poids, sur la base du poids total de la composition lubrifiante.

12. Composition lubrifiante selon l'une quelconque des revendications précédentes, dans laquelle le modificateur de viscosité semi-cristallin est compris en combinaison avec un modificateur de viscosité amorphe.

13. Composition lubrifiante selon l'une quelconque des revendications précédentes comprenant en outre un ou plusieurs des composants suivants : inhibiteurs de corrosion, inhibiteurs d'oxydation, modificateurs de frottement, dispersants.

14. Procédé de lubrification d'un moteur à combustion à allumage par compression ou à allumage par étincelle comprenant le fonctionnement du moteur avec une composition lubrifiante selon l'une quelconque des revendications précédentes.

15. Utilisation, dans une composition lubrifiante qui comprend une huile de base de groupe III API, de (b) un ou plusieurs modificateurs de viscosité semi-cristallins tels que définis dans l'une quelconque des revendications 1 à 13 ; en combinaison avec (c) un ou plusieurs LOFI tels que définis selon l'une quelconque des revendications 1 à 13, pour améliorer les propriétés d'écoulement à basse température de la composition lubrifiante.
